

# United States Patent [19]

Hodson

[11] Patent Number: 4,944,595

[45] Date of Patent: Jul. 31, 1990

[54] APPARATUS FOR PRODUCING CEMENT  
BUILDING MATERIAL

[76] Inventor: Simon Hodson, 3916 State St., Santa  
Barbara, Calif. 93102

[21] Appl. No.: 234,819

[22] Filed: Aug. 19, 1988

[51] Int. Cl.<sup>5</sup> B28C 5/16; B01F 5/12;  
B01F 7/22

[52] U.S. Cl. 366/65; 366/265;  
366/302; 366/329

[58] Field of Search 366/64, 65, 66, 67,  
366/263, 264, 265, 292, 293, 295, 302, 307, 137,  
327, 329, 330

[56] References Cited

U.S. PATENT DOCUMENTS

- 2,212,260 8/1940 Brothman ..... 366/302 X  
2,628,081 2/1953 Laird ..... 366/264  
2,882,149 4/1959 Willems ..... 366/293 X  
3,734,469 5/1973 Goldstein et al. .  
4,225,247 9/1980 Hodson ..... 366/65 X  
4,272,198 6/1981 Velikov et al. ..... 366/65  
4,552,463 11/1985 Hodson ..... 366/295

FOREIGN PATENT DOCUMENTS

2202185 7/1973 Fed. Rep. of Germany ..... 366/65

OTHER PUBLICATIONS

"Design and Control of Concrete Mixtures," Thirteenth edition by Steven H. Kosmatka and William C. Panarese, 1988, Month Unknown, Illinois at p. 96, this page makes reference to high energy mixers, the remainder of this publication describes the science of concrete.

Primary Examiner—Harvey C. Hornsby

Assistant Examiner—Scott J. Haugland

Attorney, Agent, or Firm—Spensley Horn Jubas & Lubitz

[57] ABSTRACT

A cement paste generator produces a paste with improved workability. The cement paste generator includes a housing, a shaft and a series of blades and baffles which have critical dimensions.

20 Claims, 12 Drawing Sheets



FIG. 1



0461 25KV X250 100µm WD32

FIG. 2



6731 25KV X250 100µm WD39

Fig. 3



0370 25KV X250 100µm WD32

Fig. 4



6742 25KV X250 100µm WD39

Fig. 5



Fig. 6



Fig. 7



FIG. 8



FIG. 9



Fig. 10



Fig. 11



Fig. 12



Fig. 13



*Fig. 14*  
PRIOR ART



Fig. 15



WATER-CEMENT PASTE 2" CUBE SAMPLES

Fig. 16



FIG. 17



FIG. 17



Fig. 18



Fig. 20



Fig. 19



Fig. 21



Fig. 22



Fig. 23



## APPARATUS FOR PRODUCING CEMENT BUILDING MATERIAL

### BACKGROUND OF THE INVENTION

#### 1. Field of the Invention

The present invention relates to cement paste generators.

#### 2. Description of Related Art

In the construction and building industry concrete is generally defined as a mixture of two components, aggregates and paste. The paste, which typically includes Portland cement and water, binds the aggregates (sand and gravel or crushed stone) into a rocklike mass as the paste hardens. The paste hardens because of the chemical hydration reaction between cement and water. In this regard, the technology of concrete is discussed in S. H. Kosmatka and W. C. Panarese, "Design and Control of Concrete Mixtures," 13th edition, Portland Cement Association, 1988.

The paste component of concrete, either separate from or combined with aggregate, forms a relatively continuous and consistent solid when cured. In conventional cured paste, voids or small discontinuities are normally found which have a deleterious affect on the performance characteristics of the cured paste and concrete. Commonly such limitations on performance characteristics include failure under heavy load and stress conditions.

The most common constituent of the bonding material in the concrete, i.e., that which bonds the aggregate, is Portland cement paste. The four principal chemical constituents of Portland cement are tricalcium silicate, dicalcium silicate, tricalcium aluminate and tetracalcium aluminoferrite. These components react with water (hydration) causing the setting and hardening of the cement. The process of cement hydration is characterized by the formation of a polymorphic crystalline mass as discussed below.

Studies have found that the constituents of Portland cement experience generally constituent specific partial hydration when processed by conventional means. This results in characteristic polymorphic crystalline formations of calcium silicate hydrate and calcium sulfoaluminate "ettringite" (exemplified by a needle-like structure), calcium hydroxide "Portlandite" (characterized by hexagonal crystalline plates), a spindle columnar crystal structure and an amorphous calcium silicate crystal structure. Colonies of these polymorphic crystalline mass formations are observed in random disposition relative to each other within typical cured cement pastes. This visually observably dissimilar crystallization has long been accepted and attributed to the chemical reaction between water and the tricalcium silicate, dicalcium silicate, tricalcium aluminate and tetracalcium aluminoferrite components.

One apparatus patent of particular interest to the cement paste generator of the present invention is U.S. Pat. No. 4,552,463. This patent discloses an apparatus shown generally in FIG. 14 comprising a hollow enclosure (12') having a feed inlet (14') to receive water and Portland cement to be colloidalized into a paste, and a discharge outlet (16') to dispense the colloidal paste. A rotatable drive shaft (38') is disposed along the central longitudinal axis of the enclosure. Several flat baffles (68') and (74'), disposed in planes parallel with the shaft

(38'), extend from the inner walls (76') and (78'), respectively, of the enclosure (12') towards the shaft (38').

Connected to the shaft (38') is a first upper set of downthrust blades (26') which are substantially horizontal and which thrust the mixing water and cement downward in direction "a", a second upper set of downthrust blades (28') substantially perpendicular to the first upper set of downthrust blades (26') which direct the mixing water and Portland cement inward towards the drive shaft (38') in direction "b", a lower set of downthrust blades (30') which thrust the mixing water and Portland cement downwardly and outwardly in the direction "d", a lower set of horizontal upthrust blades (34') which thrust the mixing water and Portland cement upward in direction "e" between the baffles (68') and (74'), and an upper set of upthrust blades (32'). These blades (32') are horizontal to the first upper set of downthrust blades (26') and perpendicular to the second upper set of downthrust blades (28'). In general they thrust the mixing cement and water upward in direction "e". As can be seen in the figure, the upper and lower baffles are spaced apart to create a space for receiving the upper set of upthrust blades (32').

Although the apparatus disclosed in U.S. Pat. No. 4,552,463 provides a superior paste, there is a continuing need to improve upon the paste and in particular to improve the strength and performance of the building material resulting from curing paste by conventional curing techniques. It is to this object that the present invention is directed.

### SUMMARY OF THE INVENTION

The present invention is directed to a unique cement paste generator for producing a novel paste.

By attempting to achieve substantially complete hydration by homogenous mixing of cement and water, a building material of improved strength, handling characteristics and overall performance is realized. The building material has fewer random entrapped air voids, a greater homogeneity of hydrated compounds, fewer partial or incomplete hydrated compounds, and a more fully developed homogeneous monolithic crystalline structure.

When cured and set, substantially all of the paste produced by the generator of the present invention crystallizes into a homogeneous mass of monolithic calcium silicate hydrate crystals of similar geometric configuration. Visual inspection shows that each of the monolithic masses are composed of a block of well defined plates of geometric uniformity which may be hexagonal. These well defined plate crystals are uniform and are much more fully developed and much larger than those observed in conventional partially hydrated Portland cement. The more fully crystallized plates may grow in strata-type formation to form an extremely high density matrix accounting for the decrease in the number of voids and increased strength.

A comparison between the compressive strength of cured conventional paste and the building material produced from the generator of the present invention shows such building material to be significantly stronger.

The cement paste generator of the present invention employs a hollow generally cylindrical housing. Disposed in the radial center of the housing is a rotatable shaft, having its upper end coupled to a shaft rotating mechanism. By choosing certain operating parameters and certain dimensions of the components of the gener-

ator of the present invention to be within critical ranges, the inventors have surprisingly found that a novel homogeneous paste is generated which when cured by ASTM (American Society for Testing and Materials) standards, provides a superior crystalline building material. Moreover by adding aggregates to the homogeneous paste, and then mixing again, a superior performance concrete is formed following curing.

In particular, the cement paste generator housing includes a downthrust generating component and an upthrust generating component. These components act in cooperation with a directional control means to form turbulent liquid (cement and water) mass flow patterns which move in several opposing directions relative to each other within the hollow housing.

A preferred embodiment of the inner walls of the housing of the cement paste generator of the present invention includes an upper cylindrical portion adjacent to a middle conical portion which is adjacent to a lower conical portion. The radius of the cylindrical portion and the ratios of this radius to other radial and height dimensions of the housing are critical to producing the novel paste.

The downthrust generating component within the housing includes a single upper and a lower set of downthrust blades. The upthrust generating component includes an upper and a lower set of upthrust blades.

The single upper set of substantially horizontal downthrust blades, which rotate within the cylindrical portion of the housing, are disposed in spaced relation relative to each other and are affixed to the drive shaft. The lower set of downthrust blades, which rotate within the middle conical portion of the housing, includes inclined blades disposed in spaced relation relative to each other. The lower set of downthrust blades have a trailing edge and a leading edge.

The upper upthrust blades, which rotate within the cylindrical portion of the housing, are substantially horizontal and are disposed in spaced relation relative to each other and are coupled to the outer ends of the upper set of downthrust blades.

The lower set of upper upthrust blades includes substantially vertical blades disposed in spaced relation relative to each other and affixed to the lower portion of the drive shaft. Each of these lower upthrust blades has a leading edge and a trailing edge.

The housing also includes several paired upper and lower vertically disposed baffles extending inwardly from the inner wall of the housing.

The lower end of the upper baffle of a baffle pair and the upper end of the lower baffle are spaced from each other, and the upper upthrust blade is rotatable within the baffle space. The smallest distance between the leading edge of the upper upthrust blade and the lower edge of the upper baffle is critical to producing the novel paste. In addition, the smallest distance between the trailing edge of the lower upthrust blade and the opposing free edge of the lower baffle is also critical to producing the novel paste.

#### BRIEF DESCRIPTION OF THE DRAWINGS

FIG. 1 is a photograph of conventional seven day cured mortar ASTM C109 at a magnification of 250 showing plates of calcium hydroxide.

FIG. 2 is a photograph of seven day cured mortar produced using the cement generator of the present invention ASTM C109 at a magnification of 250 showing monoliths of calcium silicate hydrate.

FIG. 3 is a photograph of conventional 28-day cured mortar ASTM C109 at a magnification of 250 showing plates of calcium hydroxide.

FIG. 4 is a photograph of 28-day cured mortar produced using the cement paste generator of the present invention ASTM C109 using the mixer of Example 2 at 500 rpm, 120 second mix time and 8 baffles, at a magnification of 250 showing monoliths of calcium silicate hydrate.

FIG. 5 is a photograph of conventional seven day cured mortar ASTM C109 at a magnification of 250.

FIGS. 6 and 7 are photographs of seven day cured mortar produced using the cement paste generator of the present invention ASTM C109, made using the mixer of Example 1 at 750 rpm, a 30 second mix time and 8 baffles, at a magnification of 250 showing the degree of plate formation. Unlike conventional material where the plates are formed from needles, the monoliths are not formed from needles in the building material of the present invention.

FIG. 8 is a photograph of conventional seven day cured mortar ASTM C109 at a magnification of 500 showing well formed calcium hydroxide plates, calcium silicate hydrate needles, ettringite needles and calcium silicate hydrate gel structure.

FIG. 9 is a photograph of seven day cured mortar produced using the cement paste generator of the present invention ASTM C109 at a magnification of 500 showing monoliths of calcium silicate hydrate.

FIG. 10 is a photograph of conventional one day cured paste ASTM C109 at a magnification of 500 showing calcium silicate hydrate needles, ettringite, amorphous formations, and calcium hydroxide plates.

FIG. 11 is a photograph of one day cured paste produced using the cement paste generator of the present invention ASTM C109 at a magnification of 500 showing calcium silicate hydrate monoliths without needles. This material was produced using the mixer of Example 1 at maximum rpm with 12 baffles and 120 second mix time.

FIG. 12 is a photograph of conventional seven day cured mortar ASTM C109 at a magnification of 2,000 showing calcium silicate hydrate needles, amorphous plates, calcium aluminum hydrate and other trace compounds.

FIG. 13 is a photograph of seven day cured mortar ASTM C109 produced using the cement paste generator of the present invention at a magnification of 2,000 showing calcium silicate hydrate monoliths, with particular focus on the initial growth of the monoliths not rising from needles. This material was produced using the mixer of Example 1 at 650 rpm, 120 second mix time and 8 baffles.

FIG. 14 is a prior art cement paste generator and particularly that of U.S. Pat. No. 4,552,463.

FIG. 15 is a comparison of the specific gravity of the crystalline building material produced using the cement paste generator of the present invention and conventional cement.

FIG. 16 is a cross-sectional schematical side view of one embodiment of the cement paste generator of the present invention.

FIG. 17 is a cross-sectional schematical view of one embodiment of the cement paste generator of the present invention showing certain dimensions.

FIG. 18 is a top view of the upper set of downthrust blades of one embodiment of the cement paste generator of the present invention.

FIG. 19 is a partial cross-sectional end view of an upper downthrust blade of one embodiment of the cement paste generator of the present invention.

FIG. 20 is a partial cross-sectional end view of an upper upthrust blade of one embodiment of the cement paste generator of the present invention.

FIG. 21 is a top view of the lower downthrust blades of one embodiment of the cement paste generator of the present invention.

FIG. 22 is a partial cross-sectional end view of a lower downthrust blade of one embodiment of the cement paste generator of the present invention.

FIG. 23 is a cross-sectional top view of the lower downthrust blades of one embodiment of the cement paste generator of the present invention.

#### DETAILED DESCRIPTION OF THE PREFERRED EMBODIMENT

The crystalline building material produced by the generator of the present invention is formed from a paste having a cement component of at least 20% and preferably 75% by weight Portland cement. After curing the paste, a substantially homogeneous mass of monolithic crystals of similar uniform geometric configuration are formed. The homogenous mass of crystals is very dense with less than 10%, and preferably less than 1% by volume, intrapred voids. This building material is produced by a novel process of mixing Portland cement and water in a cement paste generator of the present invention, as more fully described below, and curing the cement paste generated in accordance with ASTM standards.

In a preferred embodiment, the building material produced by the generator of the present invention is produced by mixing a predetermined volume of Portland cement including one or more of the following compounds: tricalcium silicate, dicalcium silicate, tricalcium aluminate and tetracalcium aluminoferrite in powder form with water in a particular water to cement ratio, and forming an cementitious paste. The water to cement ratio can range from 0.20 to 2.00.

FIGS. 8, 10 and 12 show the incomplete hydration crystalline products typically observed after curing conventional paste constituents. Conventional Portland cement polymorphic crystalline products are characterized by randomly dispersed colonies of calcium silicate hydrate, ettringite, Portlandite, columnar and amorphous crystals that are composed of tricalcium silicate, dicalcium silicate, tricalcium aluminate and tetracalcium aluminoferrite which react separately or incompletely with water. This visually observable dissimilar crystallization has long been accepted and explained in terms of the chemical reaction between tricalcium silicate, dicalcium silicate, tricalcium aluminate and tetracalcium aluminoferrite compounds, and water as discussed above. In this regard, it is believed that the cement paste generator of the present invention creates a more complete saturation of the cement grains with water by optimal fracturing of the cement grains in the presence of water into smaller particles resulting in homogenization of the calcium silicate compounds. This is antecedent to and a cause of the unique crystallization of the paste produced by the generator of the present invention (often being referred to as the calcium-silicate-hydrate (CSH) gel structure).

In conventional cured mortar, there are, among other formations, needles and plates: the needles are calcium silicate hydrate and the plates are calcium hydroxide. In

the mortar produced by the generator of the present invention there are almost no needles, and the monolithic crystals are formed of calcium silicate hydrate.

Substantially all of the paste resulting from processing Portland cement and water in the cement paste generator of the present invention crystallizes into a uniform monomorphic mass of monolithic crystals formed of plates of similar geometric configuration as shown in FIGS. 2, 4, 6, 7, 9, 11 and 13, wherein substantially means at least 30%, preferable greater than 75%, and more preferably, greater than 95% by volume. Specifically, visual inspection shows that each of the individual monolithic crystals includes a well defined block of plates of similar geometric uniformity. These well defined plate crystals are much more fully developed and are much larger than those observed in conventional partially hydrated Portland cement as shown in FIGS. 8, 10 and 12.

A comparison of FIGS. 1-13, shows three significant differences. First it is observed that the crystals produced by the generator of the present invention are substantially larger than conventional material. Second, the well-defined geometry of the crystals produced by the generator of the present invention graphically illustrates the more complete development of the crystals. Third, the more uniform geometry of the crystals produced by the generator of the present invention from a more dense packing results in a more consolidated crystalline building material.

The crystal growth that takes place in at least 1 day is characterized by a single monolithic, monomorphic material composed of crystals that have grown together as shown in FIGS. 5-7 and 11.

Extensive testing and comparative analysis has been conducted between the crystals resulting from curing conventional mortar that was made in accordance with ASTM C109 standard and the crystals resulting from curing the mortar produced by the generator of the present invention produced with a paste of initial water to cement ratios ranging from 0.30 to 0.50 and subsequently mixed with standard sand and cured in accordance with ASTM C109 standard.

Table I is a comparison of the flow and thus relative workability of mortar produced using the cement paste generator of the present invention as compared to conventional mortar produced in accordance with ASTM C109 standard. As shown, the mortar produced by the generator of the present invention has superior flow. Table II is a comparison of the compressive strength (psi) of 28 day cured cubes of conventional mortar and the mortar produced by the generator of the present invention. As shown, the mortar produced by the generator of the present invention is significantly stronger. FIG. 15 is a comparison of the specific gravity of 28 day cured paste cubes of conventional paste and the cured paste produced by the generator of the present invention. As shown, the cured paste produced by the generator of the present invention has a higher specific gravity, and preferably at least 1% higher.

The more fully developed plates of the crystals produced by the generator of the present invention may grow in a strata-type formation to form extremely high density matrixes. This accounts for the decrease in the number of voids and discontinuities, and the increased strength of the crystals produced by the generator of the present invention. This hydrated cement building material thus exhibits improved strength, workability and overall performance characteristics.

With reference to FIGS. 2, 4, 6, 7, 9, 11 and 13, it can be seen that the crystals produced by the generator of the present invention are homogeneous for a given volume, that is, there are greater than 20%, preferably greater than 75%, and more preferably greater than 95% by volume of monolithic crystals as compared to less than about 10% volume of less developed monolithic crystals in conventional crystalline material as shown in FIGS. 8, 10 and 12. On the other hand, conventional material principally consists of calcium silicate hydrate needles. In this regard, the term monolithic is generally meant to mean a unitary structure in the form of a block as compared to a needle which is generally meant to mean a slender pointed structure.

Using the crystals produced by the generator of the present invention, established design strengths have been achieved with up to 45% and commonly 10 to 20% less cement, and more than 10% greater strengths have been achieved with an equivalent cement to aggregate and water ratio as required in current practice.

Integral bonding of the building material produced by the generator of the present invention to existing concrete or mortar permits the use of thin section overlays without the necessity of additional bonding agents. In addition, a gap-grated aggregate using the hydrated cement building material produced by the generator of the present invention can produce a pervious material of high strength capable of handling water flow rates up to 20 inches per minute. This can reduce or often eliminate the need for positive drainage in retention systems and can virtually eliminate hydroplaning on concrete pavement.

In this regard, the compressive strength of the preferred building material produced by the generator of the present invention is at least 10% greater than that of conventional material for a given water to Portland cement ratio, the specific gravity of the preferred building material produced by the generator of the present invention is at least 1% greater than that of conventional material for a given water to Portland cement ratio, and the porosity of the preferred building material produced by the generator of the present invention is at least 5% less than that of conventional material for a given water to Portland cement ratio.

FIGS. 16-23 show one embodiment of the cement paste generator invention. The cement paste generator invention generally indicated as 10 includes a generally cylindrical hollow housing or enclosure generally indicated as 12 having a feed inlet generally indicated as 14a formed in the upper portion of the housing to supply dry Portland cement to the interior of the hollow housing 12, a feed inlet 14b for supplying water, a discharge outlet generally indicated as 16 formed in the lower portion of the housing to discharge the resulting paste and a longitudinally disposed rotatable shaft 28.

As shown in FIG. 16, the inner surface of the housing 12 includes a substantially cylindrical upper portion 66, a conical middle portion 68 and a conical lower portion 70.

As described more fully below, the housing 12 is configured to operatively house a thrust generating assembly and a directional control assembly to cooperatively form liquid mass flow patterns moving in various directions relative to each other within the hollow housing 12.

As previously discussed, the Portland cement paste generator invention has certain critical operating parameters and critical dimensions. If these critical param-

eters and dimensions are not employed, the specified embodiment of the generator of the present invention will not facilitate the production of the novel paste described above. As used hereinafter, use of the broadest range of the critical operating parameters and critical dimensions will provide greater than 50% by weight of the novel crystals when the paste created by the cement paste generator is cured according ASTM standards. When the preferred critical operating parameters and critical dimensions are used, greater than 9% by weight of such crystals are produced at a water to cement ratio of 0.33.

The thrust generating assembly includes a downthrust generating component and an upthrust generating component.

As shown in FIG. 16, the downthrust generating component includes a single upper set and a lower set of blades generally indicated as 18 and 20, respectively. The upthrust generating component includes an upper and a lower set of blades generally indicated as 22 and 24, respectively.

As best shown in FIGS. 16 and 18, the single upper set of downthrust blades 18 includes at least two and preferably six substantially horizontal blades 26 coupled to drive shaft 28 in spaced relation relative to each other by an upper collar 30. The outer end of each of the substantially horizontal upper downthrust blades 26 is interconnected by an upper annular support ring 32. It should be appreciated here that a substantial difference between the generator of the present invention and the apparatus of U.S. Pat. No. 4,552,463 becomes apparent in that the upper set of downthrust blades in the '463 patent includes a horizontal component (36') and a vertical component (28') which spaces the horizontal component (36') from the horizontal upper upthrust blade (32'); whereas, the present invention does not include a member equivalent to the vertical component (28') of the '463 patent nor is the upper downthrust blade 18 of the present invention substantially spaced from the upper upthrust blade 22 of the present invention. In addition, the upper upthrust blades are substantially coplanar with the upper downthrust blades. This physical configuration contributes to increasing the number of shear zones to thereby improve the characteristics of the crystals resulting from curing the novel paste described above.

As best shown in FIGS. 16, 18 and 20, the upper set of upthrust blades 22 includes at least six and preferably twelve substantially horizontal blades each indicated as 34 affixed in spaced relation relative to each other on the upper annular support ring 32. As shown in FIG. 20, each of the plurality of substantially horizontal upper upthrust blades 34 includes a leading and trailing edge indicated as 40 and 42, respectively. As discussed below, it has been discovered that the smallest distance "G1" between the leading edge 40 of the upper upthrust blade and the lower edge 62a of the upper baffle 62 is critical to the process of the present invention. Other important, but not necessarily critical dimensions include G2, the smallest distance between the trailing edge 42 of the upper upthrust blade and the upper edge 64a of the lower baffle 64, and G4, the smallest distance between the outermost end of the upper upthrust blade 34a and the cylindrical inner wall portion of the housing 66a.

As shown in FIGS. 16, 18 and 19, each of the plurality of substantially horizontal upper downthrust blades 26 is substantially pie-shaped in configuration, with

each having a leading edge and trailing edge indicated as 36 and 38, respectively.

As shown in FIGS. 16, 18 and 21, the lower set of downthrust blades 20 includes at least two and preferably six inclined blades each indicated as 44, with each including a leading edge 46 and a trailing edge 48 and having a configuration similar to that of the substantially horizontal upper downthrust blades 26. The lower portion of each inclined intermediate downthrust blade 44 is attached to the drive shaft 28 by an intermediate collar 50, and the upper portions are affixed to an intermediate support ring 52 such that the intermediate downthrust blades 44 form a substantially conical configuration relative to the drive shaft 28. As shown in FIG. 21, the upper portion of each blade 44 may be arranged to form a partial helical spiral configuration on the inside of the intermediate support ring 52. As described below, the conical plane of the intermediate downthrust blades 44 is substantially parallel to lower portion 70 of the housing 12.

To direct the vertical movement of the mixing paste, an upper and lower directional control means is provided. As shown in FIG. 16, the upper directional control means preferably includes a plurality, preferably 2-12, and more preferably 8, vertically disposed flat baffles each indicated as 62 extending radially inwardly from the housing 12. The lower directional control means includes a plurality, preferably 2-12, and more preferably 8 vertically disposed flat baffles each indicated as 64 extending radially inwardly from the housing 12.

With further reference to FIG. 17, another critical dimension is "G5", the smallest distance between the trailing edge 58 of the lower upthrust blade and the lower free edge 76 of the opposing lower baffle. Other important but not necessarily critical dimensions are "G3", the smallest horizontal distance between the trailing edge 48 of the lower downthrust blade and the outer edge of the opposing lower baffle 64, and "G6", the smallest distance between the leading edge 60 of the lower upthrust blade and the lower conical inner wall portion of the housing 70a.

As shown in FIGS. 16 and 23, the lower set of upthrust blades 24 includes at least two and preferably six flat substantially vertical blades each indicated as 54 coupled to the drive shaft 28 by lower collar 56. As shown in FIG. 16, the outer portion of each flat substantially vertical lower upthrust blade 54 includes an upper and lower edge indicated as 58 and 60, respectively, inclined relative to each other. The lower edge is preferably parallel to the lower conical wall portion 70 of the housing 12.

It should also be appreciated that when comparing the lower set of upthrust blades in the generator of the present invention with the apparatus of U.S. Pat. No. 4,552,463, it should be appreciated that the lower set of upthrust blades includes the upper and lower inclined edges 58 and 60, respectively; whereas, the lower set of upthrust blades in the '463 patent does not show or suggest such upper and lower edges. This configuration in the present invention further adds to the increased turbulence and multiplicity of mechanical and liquid shear zones which further impact upon the ability of the cement paste generator of the present invention to provide a superior Portland cement paste.

As shown in FIG. 16, the lower inclined portion 70, the inner edges 72 of the lower portion 74 of the lower baffles 64, the conical plane formed by the lower down-

thrust blades 44 and the lower edges 60 of the flat substantially vertical lower upthrust blades 54, are all substantially parallel relative to each other. Similarly, the lower edges 76 of the lower portion 74 of the lower baffles 64 are substantially parallel to the upper edges 58 of the flat substantially vertical lower upthrust blades 54.

Also with reference to FIG. 17, three radii R1, R2 and R3, three critical heights H1, H2 and H3, and two critical vertical distances H2a and H3a can be defined. Ratios of these radii, heights and vertical distances have been found to be critical to the structure of this embodiment of the present invention.

R1 is the radius of the cylindrical portion of the inner wall of the housing, R2 is the smallest radius of the middle conical portion of the inner wall of the housing within the plane containing the upper edge 54a of the lower upthrust blade, and R3 is the smallest radius of the lower conical portion of the inner wall of the housing along the plane containing the lower edge 54b of the lower upthrust blade.

H1 is the vertical distance, along the shaft, between the horizontal plane containing the leading edge of the upper upthrust blade and lower end of the cylindrical portion 66 of the housing, H2 is the distance, along the shaft 28, between the horizontal plane containing the lower end of the cylindrical portion 66 of the housing and the horizontal plane containing the lower end of the middle conical portion 68 of the housing, and H3 is the distance, along the shaft 28, between the horizontal plane containing the lower end of the middle portion of the housing 68 and the horizontal plane containing the lower end of the lower conical portion 70 of the housing.

It should be appreciated that the middle and lower conical portions can be modified and changed to a single spherical portion having the same volume. In such case H2 is defined as the smallest distance between the lowest point on the housing shaft where the inner radius is R1 and the highest point on the shaft where the inner radius is R2; and H3 is the smallest distance between the lowest point on the housing shaft where the inner radius is R2 and the highest point on the shaft where the inner radius is R3.

In general the upper downthrust/upper upthrust blade assembly must be higher than the middle downthrust blades which in turn must be higher than the lower upthrust blades. With reference to FIGS. 16 and 17, H2a is the smallest vertical distance between the height (along the shaft) containing the horizontal plane of the upper most portion of the lower downthrust blade and the horizontal plane containing the largest radius of the middle conical portion 68 of the housing. H3a is the smallest vertical distance between the bottom 80 of the mixer and the lowest portion of the lower upthrust blade.

In order to produce the novel paste of the present invention, it is necessary that the radii, height and vertical distance dimensions be chosen to be within certain critical ratios. For R1 ranging from 4.0 to 48.0 inches, it is critical that the ratio of R1 to H1 range from 0.39 to 0.45, the ratio of R1 to R2 range from 0.80 to 0.83, the ratio of R1 to H2 range from 0.59 to 0.61, the ratio of R1 to R3 range from 0.36 to 0.41, and the ratio of R1 to H3 range from 0.30 to 0.32, the ratio of R1 to H2a ranges from 0.001 to 1.0, and the ratio of R1 to H3a ranges from 0.001 to 1.0.

The gap distances G1-G6 shown in FIG. 12 constitute six mechanically induced shear zones. The gap distances are relative to the critical average blade tip velocity "S" (in feet per second) of the two upthrust blades and the two downthrust blades.

For R1 ranging from 4.0 to 48.0 inches, G1-G6 should range from 0.1 to 2.0 inches. The preferred ranges for G1-G6 are G1=0.20±0.125, G2=0.20±0.125, G3=0.20±0.125, G4=0.38±0.125, G5=0.25±0.125 and G6=0.50±0.125.

With reference to FIG. 17, it should be appreciated that angle "a" between the outer face of the support ring 32 and the trailing edge of the upper upthrust blade ranges from 45°-90°, and is preferably 80°.

For R1=8.0 inches, shaft rpm can range from 300-900, and preferably 500. For R1=24 inches, shaft rpm can range from 150-250, and preferably 165. In these preferred cases, G1-G3 are 0.20, G4 is 0.38, G5 is 0.25 and G6 is 0.50.

In addition to the critical dimensions discussed above, there are critical processing parameters. The relationship between shaft rpm and R1 must be such that the product of R1 multiplied by shaft rpm ranges from 2,000 to 7,000, with the preferred range being from 4,000 to 5,000.

The paste volume ("V") is also critical. The stationary paste volume should range from a height of 0.5H1+H2+H3 as a minimum to a height of H1+H2+H3+(4×R1) as a maximum. The preferred range is between a resting volume height on the shaft of H1+H2+H3+0.5R1 to a resting volume height on the shaft of H1+H2+H3+2.5R1.

Mix time ("MT") is relative to volume and water to cement ratio. The relationship is such that the higher the water to cement ratio the less critical the mix time, and the higher the volume the longer the mix time. In general, the paste produced by the generator of the present invention can be produced using the generator of the present invention and the rpm and volume ranges of the present invention, in a mix time ranging from 20 seconds to 300 seconds, with the preferred mix time being 60 to 120 seconds.

Water to Portland cement ("W/C") ratio ranges from 0.20 to 2.00 with a preferred range of 0.30 to 0.50. This range is using a typically available Portland cement and typically available water, but without the effect of admixtures or other chemicals. The addition of chemicals may alter the total range and/or preferred range of water to cement ratios.

It is important to note that in addition to the shearing action between the liquid masses, due to the rotational vectors created by the thrust generating assembly, the particles within each liquid mass mechanically interact. Moreover, the rotational vector created by the lower set of upthrust blades 24 causes the rotating upwardly moving liquid mass to impact against the vertically disposed lower baffles 64 directing the upwardly moving liquid mass upwardly opposite the downwardly moving liquid mass. As the upwardly moving liquid mass changes direction above the upper upthrust blades to a downward direction, the liquid mass twists and moves downward in a curling motion against the direction of the shaft rotation.

As a result of the generator of the present invention, substantially all of the cement particles are believed to be uniformly ground to an average surface area greater than that generated by conventional techniques. It is also believed that as a result of this mixing, the water

can better penetrate the cement pores leading to better hydration and crystallization.

In general, as the liquid mass moves upwardly the mechanical force of the substantially horizontal upper upthrust blades 34 draw the liquid mass upwardly. The vertical disposed upper and lower baffles 62 and 64 reduce the centrifugal or horizontal component and direct the liquid mass to enter into the mechanical influence of the substantially horizontal upper downthrust blades 34. This is continued until the desired paste is produced.

Lastly it should be appreciated that the shaft is rotated by mechanism means for rotation 78 which is apparent to those of skill in the art.

#### EXAMPLE 1

A cement paste generator was constructed wherein, in inches, R1=24.75, H1=9.75, R2=19.81, H2=14.50, R3=9.00, H3=7.50, H2a=0.11, H3a=0.02, G1-G3=0.20, G4=0.38, G5=0.25, G6=0.50, V=26.96 cubic feet and shaft rpm=165. Using W/C of 0.30 to 0.50 and MT of 60-90 seconds, the compressive strength of the cured concrete increased 15-20% as compared to conventionally batched and mixed concrete tested in accordance with ASTM C39 standard.

#### EXAMPLE 2

A cement paste generator was constructed wherein, in inches, R1=8.00, H1=3.60, R2=6.50, H2=4.90, R3=3.25, H3=2.37, H2a=0.06, H3a=0.07, G1-G3=0.20, G4=0.38, G5=0.25, G6=0.50, V=0.99 cubic feet and shaft rpm=500. Using W/C of 0.30 to 0.50 and MT of 60-90 seconds, the compressive strength of the ASTM C109 prepared mortar increased 15-20% as compared to conventionally batched and mixed mortar when tested in accordance with ASTM C109 standard.

#### EXAMPLE 3

A cement paste generator was constructed wherein, in inches, R1=24.00, H1=11.75, R2=19.81, H2=12.50, R3=9.00, H3=7.50, H2a=0.089, H3a=0.01, G1-G3=0.20, G4=0.38, G5=0.25, G6=0.50, V=26.20 cubic feet and shaft rpm=165. Using W/C of 0.30 to 0.50 and MT of 60-90 seconds, the compressive strength of the cured concrete increased 15-20% as compared to conventionally batched and mixed concrete.

It should be appreciated that although the preferred embodiment of the Portland cement paste generator of the present invention is as shown in FIGS. 16-23, other generators are within the scope of the present invention provided such generators cause the water and cement to interact such that the paste, when cured, results in the novel crystalline building material discussed above.

TABLE I

| Mortar Flow (ASTM C109) Comparison |                           |                                |
|------------------------------------|---------------------------|--------------------------------|
| Initial W/C                        | Conventional <sup>1</sup> | Present Invention <sup>2</sup> |
| 0.35                               | 93                        | 96                             |
| 0.40                               | 91                        | 95                             |
| 0.45                               | 96                        | 99                             |
| 0.485                              | 98                        | 101                            |
| Average Flow                       | 94.5                      | 97.8                           |

<sup>1</sup>Following standard mixture proportions and procedures of ASTM C109.

<sup>2</sup>Paste mixed separately in the generator of Example 2 of the present invention then brought to W/C of 0.485 for mixing with standard sand-ASTM C109.

TABLE II

| Initial<br>W/C                     | Mortar Strength Comparison<br>2" Cubes                        |                                | 5  |
|------------------------------------|---------------------------------------------------------------|--------------------------------|----|
|                                    | 28 Day Compressive Strength, psi<br>Conventional <sup>1</sup> | Present Invention <sup>2</sup> |    |
| 0.35                               | 5930                                                          | 6895                           |    |
| 0.40                               | 5840                                                          | 6735                           |    |
| 0.45                               | 6485                                                          | 7795                           |    |
| 0.485                              | 6770                                                          | 8005                           |    |
| Average<br>Compressive<br>Strength | 6256                                                          | 7358                           | 10 |

<sup>1</sup>Following standard mixture proportions and procedures of ASTM C109.<sup>2</sup>Paste mixed separately in the generator of Example 2 of the present invention then brought to W/C of 0.485 for mixing with standard sand-ASTM C109.

It will thus be seen that the objects set forth above, and those made apparent from the preceding description, are efficiently attained and since certain changes may be made in the above construction without departing from the scope of the invention, it is intended that all matter contained in the above description or shown in the accompanying drawings shall be interpreted as illustrative and not in a limiting sense.

What is claimed is:

1. In an apparatus for producing cement paste, the apparatus of the type including a hollow generally barrel-shaped enclosure having a bottom and a central longitudinally disposed rotatable shaft and having a feed inlet to receive cement and water and a discharge outlet to dispense the resulting paste, the inner wall of the enclosure including an upper cylindrical portion above and adjacent to a middle conical portion which is above and adjacent to a lower conical portion, the enclosure including a thrust generating assembly having:  
a downthrust generating component which includes a substantially horizontal set of upper downthrust blades in spaced relationship relative to each other, and a lower set of downthrust blades in a spaced relationship relative to each other, each of such blades having a leading and a trailing edge; 35  
an upthrust generating component which includes substantially horizontal upper upthrust blades in spaced relationship relative to each other, each of the upper upthrust blades having a leading and a trailing edge and being coupled to one of the substantially horizontal upper downthrust blades outwardly of the upper downthrust blades, and substantially vertical lower upthrust blades in spaced relationship relative to each other, each of such lower upthrust blades having a leading edge and a 50 trailing edge; and  
upper and lower baffles extending from the inner walls of the enclosure toward the shaft, the upper baffle having a lower end and the lower baffle having an upper end, the lower end of the upper baffle and upper end of the lower baffle being spaced from each other providing a baffle space, the lower baffle having a lower free edge, wherein each of the upper upthrust blades is rotatable within the baffle space, the improvement wherein, .  
the ratio of R1 to H1 ranges from 0.39 to 0.45, the ratio of R1 to R2 ranges from 0.80 to 0.83, the ratio of R1 to H2 ranges from 0.59 to 0.61, the ratio of R1 to R3 ranges from 0.36 to 0.41, the ratio of R1 to H3 ranges from 0.30 to 0.32, the ratio of R1 to H2<sup>a</sup> ranges from 0.001 to 1.0, the ratio of R1 to H3<sup>a</sup> ranges from 0.001 to 1.0, G1 is 0.20±0.124

inches, G5 is 0.25±0.125 inches, and V ranges from a height of H1+H2+H3 to H1+H2+H3+4R1, where R1 is the radius of the cylindrical portion of the inner wall of the housing, R2 is the radius of the cylindrical portion of the inner wall of the housing along the horizontal plane containing the upper edge of the lower upthrust blade, R3 is the radius of the lower conical portion of the inner wall of the housing along the horizontal plane containing the lower edge of the lower upthrust blade,

H1 is the distance along the shaft between the horizontal plane containing the leading edge of the upper upthrust blade and the horizontal plane containing lower end of the cylindrical portion of the housing,

H2 is the distance along the shaft between the horizontal plane containing lower end of the cylindrical portion of the housing and the lower end of the middle conical portion of the housing,

H3 is the distance along the shaft between the horizontal plane containing the lower end of the middle portion of the housing and the horizontal plane containing the lower end of the lower conical portion of the housing,

H2<sup>a</sup> is the smallest vertical distance between the upper edge of the lower downthrust blade and the plane containing the largest radius of the middle conical portion,

H3<sup>a</sup> is the smallest vertical distance between the bottom and the lower edge of the lower upthrust blade,

G1 is the smallest distance between the leading edge of the upper upthrust blade and the lower edge of the upper baffle,

G5 is the smallest distance between the trailing edge of the lower upthrust blade and the lower free edge of the opposing lower baffle, and wherein R1 ranges from 4.0 to 48.0 inches.

2. The apparatus of claim 1 wherein G2 is 0.20±0.125, G3 is 0.20±0.125, G4 is 0.38±0.125 and G6 is 0.50±0.125, wherein

G2 is the smallest distance between the trailing edge of the upper upthrust blade and the upper edge of the lower baffle,

the lower baffle having an outer edge, and G3 is the smallest horizontal distance between the trailing edge of the lower downthrust blade and the outer edge of the lower baffle,

each upper downthrust blade having a free end, and G4 is the smallest distance between the free end of the upper upthrust blade and the cylindrical inner wall portion of the enclosure, and

G6 is the smallest distance between the leading edge of the lower upthrust blade and the lower conical inner wall portion of the enclosure.

3. The apparatus of claim 2 wherein, in inches, R1=24.75, H1=9.75, R2=19.81, H2=14.50, R3=9.00, H3=7.75, G1-G3=0.20, G4=0.38, G5=0.25 and G6=0.50.

4. The apparatus of claim 2 wherein, in inches, R1=8.00, H1=3.60, R2=6.50, H2=4.90, R3=3.25, H3=2.37, G1-G3=0.20, G4=0.38, G5=0.25 and G6=0.50.

5. The apparatus of claim 2 wherein, in inches, R1=24.00, H1=11.75, R2=19.81, H2=12.50,

$R3=9.00$ ,  $H3=7.50$ ,  $G1-G3=0.20$ ,  $G4=0.38$ ,  $G5=0.25$  and  $G6=0.50$ .

6. The apparatus of claim 2 wherein each of the lower upthrust blades is flat and substantially vertical and is coupled to the shaft by a lower collar. 5

7. The apparatus of claim 6 wherein the leading and trailing edges are inclined relative to each other.

8. The apparatus of claim 1 wherein each of the upper downthrust blades is substantially horizontal and is coupled to the shaft. 10

9. The apparatus of claim 8 wherein the outer periphery of the upper downthrust blades is interconnected by an upper annular support ring.

10. The apparatus of claim 1 wherein each of the upper upthrust blades is substantially horizontal and 15 affixed to the outer portion of the upper downthrust blades.

11. The apparatus of claim 1 wherein each of the lower downthrust blades is upwardly inclined. 20

12. The apparatus of claim 11 wherein the lower portion of each of the inclined lower downthrust blades is attached to the shaft by an intermediate collar. 25

13. The apparatus of claim 12 wherein the upper portion of each of the lower downthrust blades is interconnected by an annular support ring such that the 25 lower downthrust blades form a substantially conical configuration relative to the shaft.

14. The apparatus of claim 11 wherein each of the inclined lower downthrust blades comprises a partial helical spiral configuration. 30

15. The apparatus of claim 1 wherein the hollow enclosure comprises a substantially cylindrical upper portion, an annular intermediate inclined portion and an annular lower inclined portion. 35

16. The apparatus of claim 15 wherein each lower baffle has a lower portion provided with an inner edge, wherein the lower downthrust blades form a conical plane, wherein the substantially vertical lower upthrust blades have lower edges, and wherein the annular lower inclined portion, the inner edges of the lower portion of 40 the lower baffles and the conical plane formed by the lower downthrust blades and the lower edges of the substantially vertical lower upthrust blades, are substantially parallel relative to each other.

17. The apparatus of claim 15, wherein the lower baffles have lower portions provided with lower edges and the lower upthrust blades have upper edges, and wherein the lower edges of the lower portion of the lower baffles are substantially parallel to the upper edges of the lower upthrust blades. 50

18. In an apparatus for producing cement paste, the apparatus of the type including a generally hollow enclosure having a rotatable shaft, the inner wall of the enclosure including a substantially cylindrical portion adjacent to and abutting a first substantially conical portion which is adjacent to and abutting a second substantially conical portion, the second substantially conical portion having an end extended from the point of abutment of the first and second substantially conical portions, the enclosure including a thrust generating 55 assembly having:

a downthrust generating component which includes a first set of downthrust blades, and a second set of downthrust blades, each of such blades having a first and a second edge; 65

an upthrust generating component which includes a first set of upthrust blades, each blade of the first set of upthrust blades having a first and a second

edge and being coupled to one of the blades of the first set of downthrust blades to extend outwardly of the first set of downthrust blades, and a second set of upthrust blades, each blade of the second set of upthrust blades having a first edge and a second edge; and

first and second baffles extending from the inner walls of the enclosure toward the shaft, the first and second baffles having respective ends which are spaced from each other providing a baffle space between the respective ends, wherein the first set of upthrust blades is arranged to be rotatable within the baffle space,

the improvement wherein, the ratio of  $R1$  to  $H1$  ranges from 0.39 to 0.45, the ratio of  $R1$  to  $R2$  ranges from 0.80 to 0.83, the ratio of  $R1$  to  $H2$  ranges from 0.59 to 0.61, the ratio of  $R1$  to  $R3$  ranges from 0.36 to 0.41, the ratio of  $R1$  to  $H3$  ranges from 0.30 to 0.32, the ratio of  $R1$  to  $H2a$  ranges from 0.001 to 1.0, the ratio of  $R1$  to  $H3a$  ranges from 0.001 to 1.0,  $G1$  is  $0.20 \pm 0.124$  inches,  $G5$  is  $0.25 \pm 0.125$  inches, and  $V$  ranges from a height of  $H1+H2+H3$  to  $H1+H2+H3+4R1$ ,

where  $R1$  is the radius of the substantially cylindrical portion of the inner wall of the housing,  $R2$  is the radius of the substantially cylindrical portion of the inner wall of the housing along the plane containing the first edge of the second upthrust blade,

$R3$  is the radius of the second substantially conical portion of the inner wall of the housing along the plane containing the second edge of each second upthrust blade,

$H1$  is the distance along the shaft between the plane containing the first edge of each first upthrust blade and the plane containing the point of abutment of the substantially cylindrical portion and the first substantially conical portion of the housing,

$H2$  is the distance along the shaft between the plane containing the point of abutment of the substantially cylindrical portion and the first substantially conical portion of the housing and the point of abutment of the first and second substantially conical portions of the housing,

$H3$  is the distance along the shaft between the plane containing the point of abutment of the first and second substantially conical portions of the housing and the plane containing the extended end of the second substantially conical portion of the housing,

$H2a$  is the smallest distance between the first edge of the second downthrust blades and the plane containing the largest radius of the first substantially conical portion,

$H3a$  is the smallest distance between the extended end of the second substantially conical portion and the second edge of the second upthrust blades,

$G1$  is the smallest distance between the first edge of the first upthrust blades and the end of the first baffle,

$G5$  is the smallest distance between the second edge of the second upthrust blades and the end of the second baffle, and

wherein  $R1$  ranges from 4.0 to 48.0 inches.

19. The apparatus of claim 18 wherein  $G2$  is  $0.20 \pm 0.125$ ,  $G3$  is  $0.20 \pm 0.125$ ,  $G4$  is  $0.38 \pm 0.125$  and  $G6$  is  $0.50 \pm 0.125$ , wherein

G2 is the smallest distance between the second edge of the first upthrust blades and the end of the second baffle,  
 the second baffle having an outer edge, and G3 is the 5  
 smallest distance between the second edge of the second downthrust blades and the outer edge of the second baffle,  
 each first downthrust blade having a free end, and G4 10  
 is the smallest distance between the free end of the

first upthrust blades and the substantially cylindrical inner wall portion of the enclosure, and  
 G6 is the smallest distance between the first edge of the second upthrust blade and the second substantially conical inner wall portion of the enclosure.

20. The apparatus of claim 18 wherein each of the first downthrust blades is secured with the shaft and has an outer portion extended from the shaft, and each of the first upthrust blades is secured with the outer portion of a respective one of the first blades.

\* \* \* \* \*